

# UNITED STATES PATENT OFFICE.

WILLIAM G. LINDSAY, OF NEW YORK, N. Y., ASSIGNOR TO THE CELLULOID COMPANY,  
OF NEW YORK, N. Y., A CORPORATION OF NEW JERSEY.

## SOLVENT FOR ACETYL CELLULOSE.

1,027,616.

Specification of Letters Patent. Patented May 28, 1912.

No Drawing.

Application filed August 10, 1911. Serial No. 643,374.

To all whom it may concern:

Be it known that I, WILLIAM G. LINDSAY, a citizen of the United States, residing in the city of New York, county of New York, 5 State of New York, have invented certain new and useful Improvements in Solvents for Acetyl Cellulose, of which the following is a specification.

The various compositions to which the 10 present invention relates are employed in the arts mainly as imitations of natural substances and consist of cellulose derivatives combined with or dissolved in certain other substances or menstrua, known as solvents 15 and diluents.

Although the final or useful form of the 20 different compounds is that of a solid or dried material, the different processes of conversion into this final solid form involve, as is well understood, the employment of solutions or mixtures of varying consistencies 25 as to plasticity, stiffness or fluidity, dependent generally on the proportion and kind of solvent used to the amount of cel- 30 lulose.

There are two classes of solvents,—liquid 35 solvents, of which chloroform, epichlorhydrin and acetone are good examples; and it is possible to use my new solvent with what 40 are known as solid solvents, such as camphor, for instance. The components of the mixed solvents may not necessarily be possessed of individual solvent power. As an 45 illustration, alcohol, which is practically a non-solvent in itself of nitro cellulose, forms a good solvent if either ether or camphor be mixed with it. The various applications of this important art require the employment of complex mixtures in the solvent,—single 50 substances being rarely used for such purposes. Hence, while the advancement of the art has, as is well known, depended largely on the discovery and application of new single solvent substances, it has required also the invention of combinations 55 of solvents by which effects are produced quite different from those produced when single solvents are employed alone.

My present invention relates to that kind 60 of soluble cellulose which is known as acetyl cellulose, and I have discovered that while

ethylenechlorid is not a solvent of the acetone-soluble variety of acetyl cellulose, it becomes such a solvent upon admixture either with ethyl or methyl alcohol. 55

As an illustration, I have discovered that a mixture of ethylenechlorid B. P. 83. 5° C. and methyl alcohol in the proportion of two and one-half parts of ethylenechlorid (by volume) to one part of methyl alcohol (by volume) produces a mixture which is a valuable solvent for acetyl cellulose. If the proportion of alcohol is increased beyond this amount the solvent action decreases. Again, I have found that a mixture of two and one-half parts of methyl alcohol (by volume) and one part of ethylenechlorid (by volume) produces a mixture which is a valuable solvent for acetyl cellulose, but if the proportion of ethylenechlorid is increased beyond this amount the solvent action decreases. Still again, I have found that a mixture of ethylenechlorid and ethyl alcohol in equal proportions forms an efficient solvent. But I do not limit myself to these specific proportions given in the above examples. 70 75

This new solvent mixture described herein can be used either alone or in conjunction with other solvent or non-solvent liquids or solids. 80

What I claim and desire to secure by Letters Patent is:

1. As a new composition of matter, a solution of acetyl cellulose in a mixture of ethylenechlorid and alcohol, substantially as described. 85

2. A new composition of matter consisting of a solution of acetyl cellulose in a mixture of ethylenechlorid and alcohol (ethyl or methyl), combined with other solvents, substantially as described. 90

3. A new composition of matter consisting of a solution of acetyl cellulose in a mixture of ethylenechlorid and alcohol (ethyl or methyl), combined with other solvents and inert or coloring matters and substances, substantially as described. 95

WILLIAM G. LINDSAY.

Witnesses:

J. E. HINDON HYDE,  
MABEL DENTON.